

## UNITED STATES PATENT OFFICE

2,616,867

COMPOSITION FOR AND METHOD OF  
SIZING YARNSElmer H. Rossin, Melrose, Mass., assignor to  
Monsanto Chemical Company, St. Louis, Mo.,  
a corporation of DelawareNo Drawing. Application August 30, 1950,  
Serial No. 182,399

17 Claims. (Cl. 260—29.6)

1

The present invention relates to improvements in the art of sizing water-insoluble synthetic linear polymer warp yarns such as synthetic linear polyamide warp yarns. It more particularly relates to improvements in the art of sizing polyhexamethylene-adipamide warp yarns and polyacrylonitrile warp yarns.

One of the difficulties heretofore experienced in the weaving of synthetic linear polymer yarns as, for example, polyhexamethylene-adipamide yarns and similar yarns, which stretch under slight stress and regain their original length quickly when the stress is removed, is that the size tends to dust or shed from the yarns during the weaving operation due to poor adhesion of the size with the result that the yarns are not adequately protected during weaving. Natural sizing agents such as starch or gelatin which are generally suitable for sizing cotton and regenerated cellulose yarns are not satisfactory for sizing synthetic linear polymer yarns such as polyhexamethylene-adipamide yarns.

Various water-soluble artificial polymeric materials as, for example, polyvinyl alcohol have been suggested for sizing synthetic polymer yarns but these generally are only satisfactory for sizing low twist knitting yarns. Polymethacrylic acid has been suggested heretofore as a size for polyhexamethylene-adipamide yarns but has the disadvantages of being difficultly soluble in water and also quite expensive. Also solutions of polymethacrylic acid are acidic and this makes them unsatisfactory from the standpoint of corrosion of the machinery used in sizing and weaving the yarns.

It has also been proposed heretofore to employ water solutions of quaternary ammonium hydroxide salts of styrene-maleic anhydride copolymers together with a reactive substance such as formaldehyde, alkylene polyamines or thermosetting resins for the treatment of nylon fabrics and other nylon textile materials for the purpose of producing a water resistant, permanently stiffened finish on the fabric. These quaternary ammonium hydroxide salts as a class are not satisfactory for sizing nylon textiles and they have only been useful when used in conjunction with the aforementioned reactive materials, namely, formaldehyde or the like. The use of a reactive substance with such salts, however, results in the formation of a water-insoluble resin which cannot be removed from the fabric by simple washing.

In accordance with the present invention, it is possible to size linear polymer yarns with a

2

new essentially neutral, water-soluble polymeric material which provides sized yarns having high weaving efficiency and excellent abrasion resistance.

5 It is accordingly one object of this invention to provide a novel composition for sizing water-insoluble synthetic linear polymer yarns.

A further object of this invention is to provide an improved method of sizing water-insoluble synthetic linear polymer yarns of the nature of synthetic linear polyamide yarns and polyacrylonitrile yarns.

10 15 A further object of this invention is to provide sized water-insoluble synthetic linear polymer yarns which are produced at relatively low cost and have a high weaving efficiency when woven in customary looms under normal conditions of humidity.

Still further objects and advantages of this 20 invention will appear in the following description and the appended claims.

The objects of this invention are attained, in 25 general, by first applying to the naked or presized water-insoluble synthetic linear polymer yarn as, for example, a polyhexamethylene-adipamide yarn, a water solution of a water-soluble choline salt of a copolymer consisting of the copolymerization product of an ethylene  $\alpha,\beta$  dicarboxylic anhydride or acid, or partial alkyl esters of such acid having not more than 3 carbon atoms in the alkyl group, or combinations thereof, and a polymerizable vinyl aromatic compound having a single  $>\text{C}=\text{CH}_2$  group as, for example, styrene. The solution of the choline salt of the copolymer may be slightly acid or alkaline, but, 30 preferably, should have a pH between 4.5 and 9.5. The temperature of the size solution is generally within the range of 60 to 205° F., but preferably is within the range of 130 to 150° F. After the 35 solution has been applied to the synthetic polymer yarn in a suitable manner as, for example, by passing the warp yarns through a conventional size box containing the sizing solution, the sized 40 yarns are dried to render them substantially non-tacky, preferably by passing them over heated 45 drying cans of the type conventionally employed in warp slashing machinery.

The amount of choline salt of the copolymer 50 applied to the yarn will vary to some extent depending upon the construction of the yarn and the amount of twist put in the yarn as well as the construction of the fabric, but is generally within the range of about 1 to 15% by weight based on the weight of the yarn. Best results are obtained by applying between 5 and 15% by weight of the

choline salt of the copolymer based on the yarn and such amounts are preferred.

The term "water-insoluble synthetic polymer yarn" as used herein is intended to include the water-insoluble synthetic linear polyamide yarns which show orientation along the fiber axis by characteristic X-ray diffraction patterns. As examples of such synthetic linear polyamide yarns may be mentioned polyhexamethylene-adipamide yarns and polyhexamethylenesbacamide yarns, these being preferred in this particular class of synthetic polymer yarns. Other water-insoluble synthetic linear polyamide yarns which are also satisfactorily sized in accordance with the methods of this invention are described in U. S. Patents Nos. 2,071,250, 2,130,523 and 2,130,948.

The term "water-insoluble synthetic polymer yarns" as used herein is also intended to include yarns prepared from copolymers of vinyl chloride and vinyl acetate, polyvinylidene chloride, copolymers of vinylidene chloride and vinyl chloride, and polyacrylonitrile which may contain up to 20% of a comonomer or other modifying agent, but is not intended to include yarns prepared from natural polymers such as cellulose or cellulose derivatives. Of the synthetic polymer yarns described immediately above, those prepared from polyacrylonitrile or modified polyacrylonitrile are preferably sized in accordance with the methods of this invention.

The term "yarns" as used herein is intended to include mono- or multi-filament continuous filaments, or threads or yarns containing substantial amounts, that is, from 75 to 100% of staple fibers of the polymers hereinbefore described.

The synthetic polymer yarns which are sized in accordance with the methods of this invention have a tough elastic and smooth coating thereon which coating does not substantially dust or shed from the yarns when the yarns are subsequently woven in a loom at 50 to 80% relative humidity. Woven fabrics prepared from the sized yarns are substantially free of defects normally attributable to poor sizing per se. The weaving efficiency of the sized yarns of this invention is very high and the number of yarns breaks attributable to poor sizing is reduced to a minimum. Moreover, the size is readily removed from the yarns or the woven fabric by washing the sized material in warm water or in warm water containing synthetic detergents.

The water-soluble choline salt sizing agents of this invention may be prepared in various ways. In general, they are prepared by first forming a copolymeric material by the conjoint polymerization of a polymerizable vinyl aromatic compound having a single  $>C=CH_2$  group as, for example, styrene, and an ethylene  $\alpha,\beta$  dicarboxylic acid such as maleic acid, or an anhydride of such acid such as maleic anhydride, or alkyl acid esters of such acid, for example, methyl acid maleate or mixtures of such compounds. The vinyl aromatic compound and the dicarboxylic compound or compounds are copolymerized in a mol ratio between 1:1 and 2:1 and preferably, in a mole ratio of 1:1 to 1.5:1. Although various ratios of monomers may be used to prepare the copolymer within the range described above, the copolymer will normally contain the vinyl compound and the dicarboxylic compound combined in substantially equi-molecular proportions. The resulting copolymer is then reacted in water with choline to form the choline salt, using an amount of choline sufficient to dissolve the co-

polymer in the water, and preferably to provide a solution having a pH between 4.5 and 9.5. The solutions which are slightly acidic, that is, between a pH of about 4.5 and 7.0 are highly viscous and decrease in viscosity as the pH is increased. The solutions which are alkaline reacting generally have a relatively low viscosity and decrease in viscosity with an increase in pH. In order to bring about a rapid reaction between the choline and the copolymer it is preferred to heat the water in which the reaction is carried out to a temperature of 70 to 100° C.

The copolymers employed in preparing the choline salt for sizing purposes are suitably produced by mass polymerizing the vinyl aromatic compound and the dicarboxylic compound. In the mass polymerization process, the monomeric vinyl aromatic compound and the dicarboxylic compound are generally heated to temperatures within the range of 40 to 80° C. and maintained at such temperatures until the major portion of the monomers have reacted, after which the temperature of the mass is raised to 100 to 175° C. to complete the polymerization of the remaining monomers. The mass polymerization process is preferably carried out by polymerizing the monomers in the presence of a small amount of polymerization catalyst, particularly a peroxide catalyst such as benzoyl peroxide. The mass is substantially free of solvents or diluents for the monomers. The copolymer is obtained in the form of a hard glassy resin which is preferably comminuted before it is used.

Another suitable method for preparing the copolymers for use in making the choline salt is the so-called solvent-non-solvent process which involves heating a solution of the vinyl aromatic compound and the dicarboxylic compound in a hydrocarbon liquid which is a solvent for the monomers but a non-solvent for the copolymer formed by the polymerization of the monomers. Benzene, toluene and xylene have been successfully used as the hydrocarbon liquid. The process is preferably carried out in the presence of a small amount of a polymerization catalyst, particularly a peroxide catalyst such as benzoyl peroxide. The copolymer precipitates from the hydrocarbon liquid in the form of fine particles as it is formed, and is afterwards separated from the hydrocarbon liquid by filtering or the like and then the hydrocarbon liquid is evaporated from the copolymer solids.

As examples of vinyl aromatic compounds containing a single  $>C=CH_2$  group which are useful in preparing the copolymers may be mentioned styrene, halogen substituted styrene such as p-chloro styrene, dichloro-styrene and the like, and alkyl substituted styrenes such as p-methyl styrene, dimethyl styrene and the like. Styrene is preferred because of its low cost and availability and superior properties for this particular purpose.

As examples of ethylene  $\alpha,\beta$  dicarboxylic compounds which are useful in preparing the copolymers may be mentioned maleic acid, maleic anhydride, fumaric acid, citraconic anhydride, itaconic anhydride and the like and alkyl half esters of the corresponding acids, which contain from 1 to 3 carbon atoms in the alkyl group, for example methyl, ethyl and propyl acid maleate and the corresponding fumarates, citraconates and itaconates. When the alkyl acid esters of ethylene  $\alpha,\beta$  dicarboxylic acids are used it is preferred to use a mixture of dicarboxylic compounds containing at least 50 mol per cent of an ethylene  $\alpha,\beta$  dicarboxylic acid or anhydride, more

particularly an anhydride. Maleic anhydride is the preferred dicarboxylic compound because of its low cost and ready availability and its superiority over the other dicarboxylic compounds as a component of the copolymer. Mixtures of maleic anhydride and methyl acid maleate containing from 99 to 50 mol per cent of maleic anhydride are also preferred over the other dicarboxylic compounds or mixtures thereof.

The water solution of choline salts of the copolymer are normally the sole sizing agents used in the practice of this invention. However, in some instances it is possible to use up to 20% by weight of an alkali metal salt of a styrene-maleic acid copolymer to replace a part of the choline salt. The water solutions of the choline salt of the copolymer generally contain from 4 to 35% by weight of the choline salt and have a viscosity between about 50 and 20,000 centipoises at 25° C. depending on the concentration of the solution, the pH of the solution and the particular copolymer used in preparing the choline salt. The viscosity of the solution may be modified by adding glycerine. The glycerine increases the viscosity of the solution and this is particularly desirable in some instances where the viscosity of choline salt solution is too low for sizing purposes. Amounts of 1 to 40% by weight of glycerine, on the weight of the choline salt, are generally satisfactory for this purpose. The glycerine also improves the adhesion of the size to the yarns. The solutions may also contain plasticizers such as polyethylene or polypropylene glycols and softeners such as Twitchell oil, sulfonated tallow and sulfonated vegetable oil. However, it is essential that the size solutions be free of reactive substances, that is substances which react with the choline salt at normal drying temperatures to form water-insoluble resins.

A further understanding of the methods and compositions of this invention will be obtained from the following specific examples which are intended to illustrate the invention but not to limit its scope, parts and percentages being by weight unless otherwise specified.

#### Example I

One hundred and twenty parts of a finely divided styrene-maleic anhydride-methyl acid maleate copolymer (containing 51% of combined styrene, 37.4% of combined maleic anhydride and 11.4% of combined methyl acid maleate) were added to 1188 parts of water at a temperature of 40 to 50° C. The resulting mixture was well agitated and 192 parts of a 40% water solution of choline were added. The mixture was heated to 90° C. and then boiled for one hour to dissolve the copolymer as the choline salt. The resulting solution had a pH of 7.3 (glass electrode) and a viscosity of 184 centipoises at 25° C. The solids content was 13.1%.

The solution of the choline salt as prepared above was diluted to 8% solids with water and brought to a temperature of 60° C. Unsized 70/34/7Z/100 bright, polyhexamethylene-adipamide warp yarns were passed through the solution at the rate of 12 yards per minute, and then squeezed between a rubber roll and a steel roll at a pressure of 1.66 pounds per linear inch to remove excess solution and permit penetration of the size between the filaments in the yarn. The sized yarns were then dried by passing them over five rotating drying cans heated to temperatures of 180, 200, 200, 200 and 160° F., respectively.

The dry yarns were quite supple and flexible, but yet sufficiently stiff to handle well in a loom. They were covered with a tough, elastic coating which adhered to the yarn without dusting when the yarn was quickly stretched and then immediately relaxed. After being conditioned for 24 hours at a temperature of 70° F. and a relative humidity of 65%, a number of the sized yarns were broken and the broken ends of the yarns were examined. They were found to be free of loose or fluffy filaments which indicates that the size has excellent adhesion to the yarns and also binds the individual filaments together thus affording maximum protection against yarn defects during weaving. The yarns had excellent weaving efficiency when woven in a conventional loom, and the size was readily removed from the woven fabric by washing the fabric in warm water.

#### Example II

A water solution of the choline salt of a copolymer of styrene-maleic anhydride-methyl acid maleate was prepared as described in the first paragraph of Example I except that as soon as the copolymer dissolved in the water to which the choline had been added, additional quantities of the finely divided copolymer were added to the solution in small increments until the pH of the solution was 4.5 as measured by the glass electrode. The solution was diluted with water to 8% solids and at this concentration had a viscosity of 10,500 centipoises at 25° C.

Unsized 70/34/7Z/100 bright polyhexamethylene-adipamide warp yarns were sized with the above solution using the procedure described in paragraph 2 of Example I. The dry sized yarns were considerably stiffer than those prepared in accordance with the procedure of Example I, but were similar to those yarns in weaving efficiency, ease of removal of the size and in the adhesion of the size to the individual filaments of the yarns.

#### Example III

A water solution of the choline salt of a copolymer of styrene-maleic anhydride-methyl acid maleate was prepared as described in the first paragraph of Example I and to this was added sufficient glycerine to provide 30% of glycerine on the weight of the copolymer. The solution was diluted with water to 8% solids and at this concentration had a pH of 7.3 and a viscosity of 650 centipoises at a temperature of 25° C.

Unsized 70/34/7Z/100 bright polyhexamethylene-adipamide warp yarns were sized with the above solution using the procedure described in paragraph 2 of Example I. The dry sized yarns were quite supple and flexible but yet were sufficiently stiff to handle well in a loom. The size coating on yarns was tough and elastic and adhered to the yarn without dusting or shedding when the yarn was quickly stretched and immediately relaxed. The yarns had excellent weaving efficiency and few yarn breaks were encountered during weaving. Moreover, the woven fabric was substantially free of defects.

#### Example IV

One hundred and twenty parts of a finely divided styrene-maleic anhydride-methyl acid maleate copolymer (containing 51% of combined styrene, 37.4% of combined maleic anhydride and 11.4% of combined methyl acid maleate) were added to 1188 parts of water at a temperature of

40 to 50° C. The resulting mixture was well agitated and 192 parts of a 40% water solution of choline were added after which the mixture was boiled for 1 hour to dissolve the copolymer in the form of its choline salt. The solution was cooled and sufficient choline was added to bring the pH up to 9.2, after which sufficient glycerine was added to provide 30% of glycerine on the weight of the copolymer in the solution. The solution was then diluted with water until it contained 8% copolymer solids and at this concentration had a viscosity of 263 centipoises at 25° C.

Unsized 70/34/7Z/100 bright polyhexamethylene-adipamide warp yarns were sized with the above solution using the procedure described in paragraph 2 of Example I. The dry sized yarns had properties similar to those of the sized yarns prepared as described in Example III.

#### Example V

Size solutions were prepared as described in the preceding examples except that a copolymer of styrene-maleic anhydride (containing 52% of combined styrene and 48% of combined maleic anhydride-methyl acid maleate). The resulting solutions were used to size 70/34/7Z/100 bright unsized polyhexamethylene - adipamide warp yarns using the procedure described in paragraph 2 of Example I. The resulting sized yarns had properties which were similar to the corresponding sized yarns of the preceding examples.

#### Example VI

Four hundred and fifty-two parts of a finely divided styrene-maleic anhydride-methyl acid maleate copolymer (containing 51% of combined styrene, 37.4% of combined maleic anhydride and 11.4% of combined methyl acid maleate) were added rapidly to 2548 parts of a water solution containing 298 parts of choline at a temperature of 20° C. The resulting mixture was heated to a temperature of 90° C. over a period of one hour and then maintained at that temperature for another hour, after which time the copolymer dissolved in the form of its choline salt. The resulting solution was diluted with water until it contained 18% of the choline salt of the copolymer. The pH of this solution was 7.44 (glass electrode) and the viscosity was 735 centipoises at 25° C.

Seven ends of spun yarn prepared from polyacrylonitrile staple fiber were passed at the rate of 15 yards per minute through the 18% solution of choline salt of the copolymer which was maintained at a temperature of 140 to 150° F., after which the yarns were squeezed by passing them between squeeze rolls and applying a pressure of 6.66 pounds per linear inch. About 15% of the choline salt was deposited on the yarn based on the yarn weight. The sized yarns were then dried by passing them over five rotating drying cans heated to temperatures of 180, 200, 200, 200 and 160° F., respectively.

The dry yarns were sufficiently stiffened to handle well in a loom and had excellent weaving efficiency when woven in a conventional loom. Moreover, the size coating was tough and flexible and had excellent adhesion to the yarn. The size was readily removed from the yarns by washing the woven fabric in warm water.

The sized yarns possessed increased tensile strength and excellent abrasion resistance as indicated by the following tests. A portion of one of the sized yarns was first conditioned for 24 hours at a relative humidity of 65% and a tem-

perature of 70° F. and then tested for tensile strength and abrasion resistance. A control sample of unsized yarn was conditioned and tested in the same manner. The following table shows the results obtained.

| Yarn Sample             | Tensile Strength | Abrasion Resistance |
|-------------------------|------------------|---------------------|
| Unsized                 | 0.68             | 173                 |
| Sized with choline salt | 0.73             | 1405                |

<sup>1</sup> Indicates number of cycles required in abrasion resistance tester necessary to break the yarn.

Various modifications and changes may be made in the methods and compositions set forth in the foregoing description as will be apparent to those skilled in the art to which this invention appertains without departing from the spirit and intent of this invention. It is to be understood therefore that the present invention is to be limited only by the scope of the appended claims.

What is claimed is:

1. A method of sizing water-insoluble synthetic linear polymer yarns which comprises applying to said yarns a water solution of a choline salt of a copolymer consisting of the copolymerization product of a polymerizable vinyl aromatic compound having a single  $>C=CH_2$  group and an ethylene  $\alpha, \beta$  dicarboxylic compound selected from the group consisting of ethylene  $\alpha, \beta$  dicarboxylic anhydrides, ethylene  $\alpha, \beta$  dicarboxylic acids and partial alkyl esters of said acids having not more than 3 carbon atoms in the alkyl group, and mixtures of said dicarboxylic compounds, and drying said yarn preparatory to weaving the same.

2. A method of sizing water-insoluble synthetic linear polymer yarns which comprises applying to said yarns a water solution of a choline salt of a copolymer consisting of the copolymerization product of styrene and maleic anhydride, and drying said yarn preparatory to weaving the same.

3. A method of sizing water-insoluble synthetic linear polymer yarns which comprises applying to said yarns a water solution of a choline salt of a copolymer consisting of the copolymerization product of styrene and a mixture of maleic anhydride and methyl acid maleate, said mixture containing from 50 to 99 mol per cent of maleic anhydride, and drying said yarn preparatory to weaving the same.

4. A method of sizing water-insoluble synthetic linear polyamide yarns which comprises applying to said yarns a water solution of a choline salt of a copolymer consisting of the copolymerization product of a polymerizable vinyl aromatic compound having a single  $>C=CH_2$  group and an ethylene  $\alpha, \beta$  dicarboxylic compound selected from the group consisting of ethylene  $\alpha, \beta$  dicarboxylic anhydrides, ethylene  $\alpha, \beta$  dicarboxylic acids and partial alkyl esters of said acids having not more than 3 carbon atoms in the alkyl group, and mixtures of said dicarboxylic compounds, and drying said yarns preparatory to weaving the same.

5. A method substantially according to claim 4, but further characterized in that the synthetic linear polyamide yarns are polyhexamethylene-adipamide yarns.

6. A method of sizing water-insoluble polyhexamethylene-adipamide yarns which comprises applying to said yarns a water solution of a choline salt of a copolymer consisting of the

copolymerization product of styrene and maleic anhydride, said solution being applied in an amount sufficient to provide from 1 to 15% by weight of said choline salt on the weight of the yarns, and drying said yarns preparatory to weaving the same.

7. A method substantially according to claim 6, but further characterized in that the water solution contains an amount of glycerine sufficient to increase the viscosity of the solution over and above the viscosity obtained with the choline salt per se.

8. A method of sizing water-insoluble polyhexamethylene-adipamide yarns which comprises applying to said yarns a water solution of a choline salt of a copolymer consisting of the copolymerization product of styrene and a mixture of maleic anhydride and methyl acid maleate, said mixture containing from 50 to 99 mol per cent of maleic anhydride, said solution being applied in an amount sufficient to provide from 1 to 15% by weight of said choline salt on the weight of the yarns, and drying said yarns preparatory to weaving the same.

9. A method substantially according to claim 8, but further characterized in that the water solution contains an amount of glycerine sufficient to increase the viscosity of the solution over and above the viscosity obtained with the choline salt per se.

10. A method of sizing water-insoluble polyacrylonitrile yarns which comprises applying to said yarns a water solution of a choline salt of a copolymer consisting of the copolymerization product of a polymerizable vinyl aromatic compound having a single  $>C=CH_2$  group and an ethylene  $\alpha,\beta$  dicarboxylic compound selected from the group consisting of ethylene  $\alpha,\beta$  dicarboxylic anhydrides, ethylene  $\alpha,\beta$  dicarboxylic acids and partial alkyl esters of said acids having not more than 3 carbon atoms in the alkyl group and mixtures of said dicarboxylic compounds.

11. A method of sizing water-insoluble polyacrylonitrile yarns substantially according to claim 10, but further characterized in that the copolymer consists of the copolymerization product of styrene and maleic anhydride.

12. A method of sizing water-insoluble polyacrylonitrile yarns substantially according to claim 10, but further characterized in that the copolymer consists of the copolymerization product of styrene and a mixture of maleic anhy-

dride and methyl acid maleate, said mixture containing from 50 to 99 mol per cent of maleic anhydride.

13. A choline salt of a copolymer consisting of the copolymerization product of a polymerizable vinyl aromatic compound having a single  $>C=CH_2$  group and an ethylene  $\alpha,\beta$  dicarboxylic compound selected from the group consisting of the ethylene  $\alpha,\beta$  dicarboxylic anhydrides, ethylene  $\alpha,\beta$  dicarboxylic acids and partial alkyl esters of said acids having not more than 3 carbon atoms in the alkyl group and mixtures of said dicarboxylic compounds.

14. A choline salt of a copolymer consisting of the copolymerization product of styrene and maleic anhydride.

15. A water solution of a choline salt of a copolymer consisting of the copolymerization product of styrene and maleic anhydride, said solution containing sufficient glycerine to increase the viscosity of the solution over and above the viscosity obtained with the choline salt per se.

16. A choline salt of a copolymer consisting of the copolymerization product of styrene and a mixture of maleic anhydride and methyl acid maleate, said mixture containing from 50 to 99 mol per cent of maleic anhydride.

17. A water solution of a choline salt of a copolymer consisting of the copolymerization product of styrene and a mixture of maleic anhydride and methyl acid maleate, said mixture containing from 50 to 99 mol per cent of maleic anhydride, said solution containing sufficient glycerine to increase the viscosity of the solution over and above the viscosity obtained with the choline salt per se.

ELMER H. ROSSIN.

#### REFERENCES CITED

The following references are of record in the file of this patent:

#### UNITED STATES PATENTS

| Number    | Name          | Date         |
|-----------|---------------|--------------|
| 351,890   | Waite         | Nov. 2, 1886 |
| 2,286,062 | Condo et al.  | June 9, 1942 |
| 2,469,407 | Powers et al. | May 10, 1949 |

#### FOREIGN PATENTS

| Number  | Country | Date          |
|---------|---------|---------------|
| 726,670 | Germany | Oct. 17, 1942 |

#### OTHER REFERENCES

Karrer, Organic Chemistry, 2nd ed., pages 234-235.